

4  
UNITED STATES PATENT OFFICE.

JOSEPH L. K. SNYDER, OF CLEVELAND, OHIO, ASSIGNOR TO NATIONAL CARBON COMPANY, OF CLEVELAND, OHIO, A CORPORATION OF NEW JERSEY.

## PROCESS OF TREATING THE SURFACE OF ARTICLES MADE OF CURED CARBON. 2197

1,178,546.

Specification of Letters Patent. Patented Apr. 11, 1916. X2261

No Drawing.

Application filed September 23, 1910. Serial No. 583,446. X3406

*To all whom it may concern:*

Be it known that I, JOSEPH L. K. SNYDER, a citizen of the United States, residing at Cleveland, in the county of Cuyahoga and State of Ohio, have invented a certain new and useful Improvement in Processes of Treating the Surface of Articles Made of Cured Carbon, of which the following is a full, clear, and exact description.

10 Articles made from carbon and cured by heat have a very hard, smooth, dense external shell or skin. There are many uses for which said carbon articles are adapted, which require the application of some surface coating. It is very difficult, however, to cause such coating to adhere suitably to the smooth, dense external skin of the article.

This invention relates to a process for 20 overcoming this difficulty, and consists in making the skin more porous by dipping in a suitable liquid agent, heating the article to drive out the volatile part of said agent, and then applying the coating. I have 25 found that either an acid, such as sulfuric acid, or an alkali, such as caustic soda solution, will make the skin of the article porous when used as the liquid agent in the process described. I am unable to advance a theory

for the phenomena, but the fact remains 30 that carbon articles are made porous by the treatment. After having opened the pores of the article the coating that is to be applied to the carbon article adheres tenaciously, as the same enters the minute 35 interstices in the skin.

A preferred way for carrying out the process is to dip the carbon article in the solution for about 30 seconds, removing it therefrom, and covering it with hot coke to 40 drive off the volatile part of the liquid, though the heating obviously may be carried on in other ways.

Having described my invention, what I claim is:— 45

1. The process of coating carbon articles, which consists in opening the pores in the skin and then applying the coating.

2. The process of coating carbon articles, which consists in dipping the article in a 50 liquid such as an acid or an alkali, heating the article and then applying the coating.

In testimony whereof, I hereunto affix my signature in the presence of two witnesses.

JOSEPH L. K. SNYDER.

Witnesses:

E. L. THURSTON,  
H. R. SULLIVAN.

Copies of this patent may be obtained for five cents each, by addressing the "Commissioner of Patents, Washington, D. C."

R.23

H